

## UNITED STATES PATENT OFFICE

2,388,047

## LUBRICATING OIL

Elliott Alfred Evans and John Scotchford Elliott,  
Beaconsfield, England, assignors to C. C. Wake-  
field & Company Limited, Beaconsfield, Eng-  
land, a British company

No Drawing. Application April 16, 1943, Serial No.  
483,336. In Great Britain April 2, 1942

16 Claims. (Cl. 252—48.6)

This invention is for improvements in or relating to lubricants which are to be used under conditions which tend to disrupt the lubricant film, which disruption more particularly takes place when the pressure between the bearing surfaces is very great.

Where the lubricant is required to lubricate surfaces under the above conditions, the film-rupture strength becomes more important than the coefficient of friction. For example, under the extreme pressures obtaining in hypoid gears, if the oil film is ruptured the metal surfaces will contact one with the other, thereby leading to loss of efficiency, excessive wear and failure of the mechanism.

There have already been provided lubricants which have a high film-rupture strength. Such lubricants are generally known in the trade as "extreme-pressure" lubricants.

These extreme-pressure lubricants originally consisted of lubricating oil which contained sulphur, either in the form of flowers of sulphur or as a colloidal dispersion. The sulphur, however, was liable to precipitation and it was later proposed to prepare these extreme-pressure lubricants by treating a fatty oil, for example an animal oil, with thionyl-chloride or with similar reagents, such as sulphur monochloride, sulphur dichloride, etc., and then adding the product of this reaction to a mineral oil.

A theory as to the action of extreme-pressure lubricants has been that the sulphur reacts with metallic surfaces and forms a very thin coating of iron sulphide and that this sulphide film is sufficient to prevent the metallic surfaces coming into contact with one another should the lubricant film be ruptured. If this theory is, in fact, correct, then it is obvious that the sulphur contained in the oil must be in such form as to be capable of reacting with the metallic surfaces which it is desired to lubricate. On the other hand, the sulphur compound must not be so reactive as to induce corrosion of the surfaces.

It was found, however, that with these prior processes no set conditions could be determined which would ensure a uniform product always being obtained and it was therefore always necessary when preparing an extreme-pressure lubricant to apply the method of trial and error in arriving at a satisfactory composition.

The present invention is a development from that described in United States Patent No. 2,164,383.

It is a further object of this invention to provide extreme-pressure lubricants which though

they may contain a substantial quantity of "active" sulphur, i. e. sulphur which will react chemically with metals such as copper at high temperatures, yet are relatively noncorrosive towards metals, especially copper, in practice under the conditions in which they are used.

It is a further object of this invention to provide new sulphur-containing addition agents for extreme-pressure lubricants, characterised by imparting a high film rupture strength to the oil in which they are dissolved together with little corrosive action on metal surfaces.

According to this invention an extreme-pressure lubricant comprises a lubricating oil having dispersed therein an aromatic hydroxy-substituted polysulphide comprising an ester substituent.

Said polysulphide comprises two aromatic radicals each of which contains both a hydroxyl and an ester substituent. Preferably the hydroxyl substituent in each aromatic radical is located in the para position to the polysulphide group.

More specifically the invention contemplates the use of disulphides, trisulphides and tetrasulphides and of mixtures of such polysulphides in varying amount, and also of mixtures of such polysulphides with varying amounts of the corresponding thioether and of minor amounts of free sulphur.

The formulae for typical disulphide, trisulphide and tetrasulphide compounds are as follows, although tri- and tetra-sulphides having other arrangements of sulphur atoms may exist:



The following procedure was adopted for determining the amount of elementary sulphur present in the solid addition agents hereinafter described.

An accurately-weighed quantity of the solid (about 1 gram) was dissolved in 20 cc. tetrahydronaphthalene in a 100 cc. beaker, and a weighed amount of copper powder (about 3 grams) was added. The beaker was placed in

an oven at 100° C. and removed after half an hour.

The copper powder was then washed into a weighed filter paper which was well washed with ether to remove tetrahydronaphthalene, dried in an oven at 100° C. and reweighed.

It was found that by this method the whole of the elementary sulphur present in any such mixture could be determined with reasonable accuracy, whereas the short time of heating did not cause appreciable decomposition of the higher polysulphides.

By employing the method of Ormandy and Craven (described in the Journal of Industrial and Engineering Chemistry, 1927, page 1281) i. e. shaking a solution of the material with mercury until formation of mercury sulphide ceased, the whole of what may be termed the "loosely held" sulphur was removed, although the time of shaking required was two days instead of half an hour. This "loosely held" sulphur is believed by us to consist of sulphur atoms combined in the form of trisulphide and tetrasulphide. In addition, of course, the free sulphur is also removed.

After the removal of all the "loosely held" and free sulphur in this way from a known amount of the material in solution, the disulphide present was reduced to mercaptan with zinc dust and acetic acid, and the mercaptan removed by shaking with 50% alcoholic plumbite solution. The residual sulphur content of the solution was then determined.

A rough confirmation of the amount of disulphide was obtained by the method of Bond (Journal of Industrial and Engineering Chemistry, Analytical, 1933, page 257).

#### Example 1

A mixture of 20.2 grams of methyl salicylate, 9.1 grams of sulphur monochloride and 2.12 grams of flowers of sulphur was warmed gently and a small amount of copper powder added.

A vigorous reaction ensued during which the sulphur dissolved. After heating for ten minutes at 120° C. the product was allowed to cool and set to a hard yellow solid.

It is believed that the reactions involved are similar to those already outlined, but that some of the added sulphur takes part in the reaction causing an increase in the amounts of tri- and tetrasulphides and a corresponding decrease in the amount of disulphide produced.

An analysis, similar to that heretofore described, indicated the following approximate composition:

|                                                           | Per cent |
|-----------------------------------------------------------|----------|
| Di(3-carbomethoxy-4-hydroxyphenyl) tri- and tetrasulphide | 40-50    |
| Di(3-carbomethoxy-4-hydroxyphenyl) disulphide             | 20-30    |
| Di(3-carbomethoxy-4-hydroxyphenyl) thioether              | 20-30    |
| Elementary sulphur                                        | 6        |
| ("Loosely held" sulphur)                                  | 10       |

#### Example 2

Methyl salicylate (60.8 grams—1 mol.) was mixed with 32.4 grams (0.6 mol.) of sulphur monochloride and 15.2 grams (1.2 gm.—atoms) of sulphur were added.

A little copper powder was added, and the reaction started by gentle warming.

After the reaction had been completed as before the product was cooled, and set to an opaque yellow plastic solid.

Such plastic characteristics may be imparted to any of these products by employing more than the theoretical quantity of sulphur monochloride, thus giving rise to secondary reaction products.

5 An analysis of this material indicated the following composition:

|                                                           | Per cent |
|-----------------------------------------------------------|----------|
| Di(3-carbomethoxy-4-hydroxyphenyl) tri- and tetrasulphide | 50-60    |
| 10 Di(3-carbomethoxy-4-hydroxyphenyl) disulphide          | 5-10     |
| 15 Di(3-carbomethoxy-4-hydroxyphenyl) thioether           | 20-30    |
| Elementary sulphur                                        | 11.5     |
| (“Loosely held” sulphur)                                  | 13.5     |

It will be understood that in this list, the polymers and secondary reaction products are included with the simple compounds.

20 A varying degree of chlorination also takes place during these reactions. Thus the material prepared as outlined in this example contained 9% of chlorine.

Whereas the formulae for the tri- and tetrasulphides have been written in the manner shown, 25 we do not wish to be restricted in any way, as the actual mode of attachment of the sulphur atoms is not known with certainty.

The products of this invention are extremely 30 effective for increasing the film-rupture strengths of lubricating oils, e. g. mineral lubricating oils.

In the following table, the effect of typical materials on the film-rupture strength (F. R. S.) of a paraffinic mineral oil is shown.

35 The testing machine employed was the well-known Almen machine.

|                      | Material added to oil | Percentage present | F. R. S. (lbs. per sq. in.) |
|----------------------|-----------------------|--------------------|-----------------------------|
| 40 Blank test        |                       |                    |                             |
| Product of Example 1 |                       | 1.0                | More than 4,000             |
| Product of Example 2 |                       | 1.0                | More than 15,000            |

45 It will be seen from the foregoing table that the products of this invention are eminently suitable extreme-pressure agents. We believe that the extreme-pressure activity of these materials is due to a combination of desirable features, viz. the presence of firmly-bound sulphur rendered active by the presence of electronegative groups, the presence of "loosely held" sulphur, and the presence of the ester groups themselves. Thus in general the compounds of this invention impart a higher film-rupture strength to oils in which they are dissolved than the corresponding polysulphides made from phenols.

50 Some of the materials contemplated in this invention contain as has already been shown minor amounts of free sulphur. Although this assists in producing a high film-rupture strength of the oil in which the material is dissolved, it is undesirable on account of its corrosive propensities, particularly towards copper and its alloys. Accordingly it is desirable to have as much "loosely held" sulphur and as little free sulphur as possible. In any case the free sulphur should not exceed about 15% of the total composition.

55 If desired, the free sulphur may be removed, 60 at least in part, by maintaining the material at a temperature just above its melting point, and allowing the sulphur to settle out, but it is not in general necessary to do this.

65 A simple test which is recognised as giving a 70 good indication of the corrosiveness of an oil

towards copper when in use consists in heating a strip of copper foil, polished with carborundum powder in 100 grams of the oil at 100° C. for one hour.

The following table indicates the superiority of oils containing our materials over oils containing elementary sulphur in the same amounts as the "active sulphur" introduced in our addition agents.

| Material and quantity added to oil | Resulting percentage sulphur in oil |          | Appearance of copper                                    |
|------------------------------------|-------------------------------------|----------|---------------------------------------------------------|
|                                    | (a) "Active"                        | (b) Free |                                                         |
| 1% product of Example 1.           | 0.16                                | 0.06     | Thin black film, giving purplish appearance to surface. |
| 1% product of Example 2.           | 0.25                                | 0.10     | Similar, but with patches of deeper black.              |
| 0.076% sulphur.                    | 0.076                               | 0.076    | Deep black.                                             |
| 0.16% sulphur.                     | 0.16                                | 0.16     | Deep black, some copper sulphide having flaked off.     |

These results would indicate not only the advantage of having as much of the "active" sulphur as possible chemically combined, but also that the polysulphides of this invention exert a highly beneficial inhibitory influence at the metal surface.

In preparing lubricating oils for extreme-pressure purposes we may employ any of the compounds of this invention or mixtures thereof in a concentration of 5% or less, and preferably 0.5 to 2%, or we may employ mixtures of these materials with the compounds of Patent No. 455,235 (e. g. di(3-carbomethoxy-4-hydroxyphenyl) thioether).

Excellent results are also obtained by employing mixtures of these compounds with halogenated organic compounds, e. g. chlorinated paraffin wax and other hydrocarbons, halogenated quinones and the nitro-polychlor-benzenes.

In one example a blend of a mineral oil, classification 90 (Society of Automotive Engineers) containing one per cent of the product of Example 2 and eight per cent of a chlorinated paraffin wax containing about 40% chlorine, when tested on the well-known Society of Automotive Engineers machine at 1,000 R. P. M. and standard rubbing ratio of 14.8, the rate of loading being 83.5 lbs./second, withstood loads up to 460 lbs.

The normal requirement for a good extreme-pressure oil of this type is that it should withstand loads upon to 325 lbs. under these conditions.

It will be understood that the materials of this invention may be added to mineral oils which may be paraffinic, naphthenic or asphaltic in type, or which may contain varying amounts of fatty oils (e. g. animal, vegetable and fish oils) or known addition agents such as pour point depressants, viscosity index improvers, anti-oxidants, sludge dispersers and detergents and corrosion inhibitors such as mercaptobenzothiazole.

We claim:

1. An extreme-pressure lubricating composition comprising a lubricating oil base having dispersed therein a reaction product of sulphur monochloride and sulphur with an aromatic hydroxy-sub-

stituted ester, said reaction product comprising a substantial proportion of aromatic hydroxy-substituted polysulphide containing at least three sulphur atoms to the molecule and having an ester substituent, said reaction product being in sufficient amount to substantially increase the film-rupture strength of said lubricating oil base.

2. An extreme-pressure lubricating composition comprising a lubricating oil base having dispersed

10 therein a reaction product of sulphur monochloride and sulphur with an alkyl salicylate, said reaction product comprising a substantial proportion of hydroxyphenyl polysulphide containing at least three sulphur atoms to the molecule and having an ester substituent, said reaction product being in sufficient amount to substantially increase the film-rupture strength of said lubricating oil base.

15 3. An extreme-pressure lubricating composition as claimed in claim 1 in which the aromatic hydroxy-substituted polysulphide comprises two aromatic radicals each of which contains both a hydroxyl substituent and an ester substituent.

4. An extreme-pressure lubricating composition 20 as claimed in claim 1 in which the hydroxyl substituent is located in the para position to the polysulphide group.

5. An extreme-pressure lubricating composition 25 as claimed in claim 1 in which the aromatic hydroxy-substituted polysulphide is admixed with the corresponding thioether.

6. An extreme-pressure lubricating composition 30 as claimed in claim 1 in which the aromatic hydroxy-substituted polysulphide is associated with minor amounts of free sulphur.

7. A process for producing an extreme-pressure lubricating composition which comprises reacting sulphur monochloride and sulphur with an aromatic hydroxy-substituted ester to 40 form a reaction product comprising a substantial proportion of aromatic hydroxy-substituted polysulphide containing at least three sulphur atoms to the molecule and having an ester substituent, and dispersing a sufficient amount of said reaction product in a lubricating oil base to substantially increase the film-rupture strength of the oil base.

8. A process for producing an extreme-pressure lubricating composition which comprises reacting sulphur monochloride and sulphur with an alkyl salicylate to form a reaction product comprising a substantial proportion of hydroxyphenyl polysulphide containing at least three sulphur atoms to the molecule and having an ester substituent, and dispersing a sufficient amount of said reaction product in a lubricating oil base to substantially increase the film-rupture strength of the oil base.

9. The composition as defined in claim 1 further characterized in that said reaction product is dispersed in the lubricating oil base in the amount of from about 0.5% to about 5%.

10. The composition as defined in claim 2 further characterized in that said reaction product is dispersed in the lubricating oil base in the amount of from about 0.5% to about 5%.

ELLIOTT ALFRED EVANS.  
JOHN SCOTCHFORD ELLIOTT.